

3,321,287

 METHOD OF IMPREGNATING LUBRICANT  
INTO ABRASIVE WHEELS

Jesse F. Hunsberger, Pottstown, and Donald J. Tucker, Huntingdon Valley, Pa., assignors to A. P. de Sanno & Son, Inc., Phoenixville, Pa., a corporation of Pennsylvania  
No Drawing. Filed July 20, 1964, Ser. No. 383,926  
1 Claim. (Cl. 51—295)

The present invention relates to abrasive grinding wheels and other abrasive tools containing a solid lubricant and to methods for increasing the permanence of the retention of solid lubricant therein.

A purpose of the invention is to permanently retain in the pores of an abrasive tool, such as a grinding wheel, a solid lubricant such as graphite, by introducing with, or after, the introduction of the solid lubricant a resinous bonding material for retaining the lubricant.

A further purpose is to impregnate an abrasive wheel such as an abrasive grinding wheel, with a solid lubricant in a suitable medium, and to introduce with, or after, the introduction of the solid lubricant, a resinous bond which will hold the solid lubricant in the pores of the tool.

A further purpose is to introduce a solid lubricant with a resinous bond in making an abrasive wheel, the resinous bond retaining the solid lubricant in place in the pores of the wheel.

Further purposes appear in the specification and in the claim.

It has been found in the prior art that certain materials can be introduced into the pores of abrasive tools such as grinding wheels, and cause the tool to run cool. They function in addition to a liquid coolant such as water, an alkaline solution, an oil, or an oil emulsion.

A reason for this extraordinary property is not fully understood, but the fact is well established.

Typical of the most widely used of these solid lubricants is graphite. To some extent, as later explained, the chlorinated naphthalenes which are of waxy consistency, such as tetra-, penta- and hexachloronaphthalene, possess the properties of solid lubricants.

Difficulty has been encountered with graphite in that it is washed out of the pores of the wheel by the liquid coolants during service, and therefore the effectiveness of the wheel is greatly reduced after a period of service.

We have discovered that it is possible to introduce a solid lubricant such as graphite and to retain this material permanently in the abrasive wheel by introducing a resinous bond. We also have discovered that the resinous bond does not impair the functioning of the solid lubricant, but leaves it in a form which is capable of effectively cooling the wheel.

The invention, while primarily intended to be used with vitrified bonded abrasive wheels, can be applied equally well to abrasive wheels and other tools having one of the other usual types of bond, such as resinous bonded, shellac bonded, magnesium oxychloride bonded, sodium silicate bonded, and rubber bonded wheels.

The resinous bond can be introduced with the solid lubricant or after introducing the solid coolant. The solid lubricant can also be introduced with the bond which forms the wheel itself if no high temperature is involved in forming the bond which would destroy the resinous bond. The resinous bond is, where possible, cured in place.

## EXAMPLE 1

For convenience in comparing the properties of the different wheels, the various examples employ aluminum oxide abrasive grit of 36 mesh size.

In this example a vitrified bonded abrasive wheel was bonded with a conventional vitrified bond consisting of

clays, feldspars and frits totalling 14% based on the weight of the wheel. The wheel was molded using conventional vitrified bonding molding technique and was then fired at a temperature of 2280° F.

After the wheel had cooled, it was treated by dipping in a dispersion of graphite lubricant and resinous bond as follows:

|                                                       | Percent |
|-------------------------------------------------------|---------|
| Dispersion of graphite powder 7% in isopropyl alcohol | 85      |
| Liquid A stage phenol-formaldehyde resin              | 15      |

The graphite powder was obtained according to the teaching of J. L. King, U.S. Patent 2,986,519, granted May 31, 1961, for Process of Forming a Graphite Lubricant.

The A stage phenol-formaldehyde resin had the following characteristics:

## Monsanto 482

|                                                         |                        |
|---------------------------------------------------------|------------------------|
| 20 Solids content                                       | 66 to 71% by weight.   |
| Viscosity                                               | 335–385 cps. at 25° C. |
| Polymerization test for dry rubber at 150° C. SDP-509-1 | 100 seconds minimum.   |
| Specific gravity at 25° C.                              | 1.180–1.200.           |
| 25 Water content                                        | 4% maximum.            |
| Free formaldehyde content                               | 1.5% maximum.          |
| pH                                                      | 5.7 to 6.2.            |

The dispersion of graphite and A stage phenol-formaldehyde resin was placed in a vessel and vitrified bonded abrasive wheels were submerged in the solution for a few minutes until all bubbling ceased.

The wheels were then removed from the solution and allowed to drain. Where the wheels were of large diameter they were rotated at low speed, approximately 1000 r.p.m., to insure good distribution of the lubricant and carrier throughout the wheels to insure homogeneity. This is done with wheels which are of six inches in diameter or larger.

After drying, the wheels were cured in an oven at 220° F. for two hours and at 350° F. for two additional hours.

The wheels were found to grind effectively and remain cool, and the lubricant remained in place throughout the service of the wheels.

## EXAMPLE 2

In this example grinding wheels of the same character were used. Instead of 15% of phenol-formaldehyde liquid resin, in this case 15% of an epoxy liquid resin formulation consisting of the following was employed:

|                                                                             | Percent |
|-----------------------------------------------------------------------------|---------|
| Liquid epoxy resin condensation product of bis phenol-A and epichlorohydrin | 66 2/3  |
| Polyamide activator                                                         | 33 1/3  |

The liquid epoxy resin condensation product of bis phenol-A and epichlorohydrin is made according to U.S. Patent 2,705,223 assigned to General Mills. The liquid resin has the following characteristics.

|                     |                             |
|---------------------|-----------------------------|
| 60 Specific gravity | 1.17 at 23° C.              |
| Viscosity           | 13,000 cps. at 23° C.       |
| Epoxy value         | 0.523 equivalents per gram. |
| Flash point         | 249° C.                     |

The reaction of bis phenol-A in order to form the condensation product is shown in Reaction I. Where  $n$  is 0 the molecular weight is about 340 and where  $n$  is 10 the molecular weight is about 3,000. In the particular product used the molecular weight was 380, obtained by use in excess of two mols of epichlorohydrin to one mol of bis phenol-A, the reaction being carried out in an autoclave in the presence of an alkaline catalyst such as sodium hydroxide.

### *Reaction 1*



Reaction 2 shows the production of the polyamide activator used in Example 2. 9, 2 linoleic acid and 9, 11 linoleic acid (isomerized) are reacted according to well known practice to form linoleic acid dimer.

As shown in Reaction 3, linoleic acid dimer reacts with a diamine such as ethylene diamine, also according to well known practice to form the polyamide activator referred to in Example 2. The properties of the polyamide activator are as follows:

Amine value ----- 290 to 320.

### Condition of fluid:

Viscosity ----- 80 to 120 poises at 40° C.

Specific gravity ----- 0.97.

In manufacturing the polyamide activator the ingredients are blended in an autoclave at low temperature and the temperature is gradually raised high enough so that water distills off from the reaction at a rate which maintains the temperature near 100° C. When distillation becomes negligible, temperature is raised from 150 to 250° C. and vacuum is applied. Reaction can be carried on in xylene as a solvent.

The following U.S. patents of General Mills describe the production of the polyamide: 2,379,413 and 2,705,223.

### *Reaction 2*



### Reaction 3



Where  $R = H$  or another linoleic dimer

Reaction 4 shows the reaction between the liquid epoxy resin condensation product and the polyamide activator 75

in Example 2. In Reaction 4, R is an alkyl group, straight or branched, or an unsaturated alkylene, straight or branched carbon chain having one to fifteen carbon atoms. R' is as shown in Reaction 1, in which  $n$  may vary from zero to fifteen and the molecular weight may vary between 100 and 5000.

20 In this case the graphite dispersion was dispersed in a solvent mixture of 40% of methylethylketone, 20% of isopropyl alcohol and 40% of toluene by volume.

The procedure of Example 1 was followed, except that the wheels after impregnation were cured at a temperature of about 250° F. for a time of one to two hours.

It was found that the lubricant functioned effectively and remained in place in the wheels.

### EXAMPLE 3

30 The procedure of Example 1 was followed, except that instead of 15% of phenol-formaldehyde A stage liquid resin, 15% of polyurethane liquid resin was used having the following composition:

35 100 parts by weight of polyurethane prepolymer.  
10 parts by weight of polyol, in this case triisopropano-  
amine.

Reaction 5 shows the general reaction between an isocyanate and an alcohol to form urethane. In Reaction 5, the isocyanate can be toluene diisocyanate, hexamethylene diisocyanate, di-phenylmethane diisocyanate, the dimethyl derivative thereof, 1,5-naphthalene diisocyanate, triphenyl methane triisocyanate, xylene diisocyanate, or the dimethyl derivative thereof, or chlorophenyl-3-4-diisocyanate. In Reaction 5 R' may be hydrogen or an alkyl group having from 1 to 35 carbon atoms in the carbon chain, or a similar alkylene group, or a corresponding hydroxylated group.

Reaction 6 shows the general reaction for forming a urethane polymer. In Reaction 6 R' will correspond to any of the isocyanates referred to in Reaction 5. R in Reaction 6 will correspond to any of the groups which constituted R' in Reaction 5.

Reaction 7 shows a general reaction for producing a polyurethane prepolymer by reacting toluene diisocyanate with a polyol. In Reaction 7 and also Reaction 8, R' may be any alkyl group having from 1 to 35 carbon atoms or a corresponding unsaturated or alkylene group or a substituent thereof substituted, for example, by hydroxyl or amine.

### Reaction 4





made into a resinous bonded wheel by typical technique of which the following is an example:

|                                                   | Percent |
|---------------------------------------------------|---------|
| Abrasive grain -----                              | 75      |
| Solid B stage phenol-formaldehyde resin powder -- | 18.7    |
| A stage phenol-formaldehyde liquid resin -----    | 6.3     |

The wheel is molded and cured suitably at 325° F. for 27 to 42 hours, in this case 27 hours.

Using grain coated with graphite, similarly any other type of wheel bonding, such as shellac, magnesium oxychloride, sodium silicate, or rubber, can be applied.

The abrasive grains employed may be of any suitable character, whether natural or synthetic. Among the natural abrasive grains which can be used are corundum, emery or sand. Among the synthetic abrasive grains which will be used are aluminum oxide, silicon carbide, zirconium spinel, titanium spinel, various metal nitrides, and diamonds.

In experimental work using wheels produced according to the invention, it is found that various advantages exist. The wheel has 25% more life before dressing and retains this characteristic indefinitely.

The wheel increases the number of pieces ground by about 25% and this continues throughout the life of the wheel.

The metal finish obtained is 50% better and this remains as a characteristic of the wheel.

There is less loading of metal particles in the wheel.

The over-all wheel life is increased.

The tendency to form heat checks on the work pieces is greatly reduced.

The quantity of solid lubricant such as graphite on the weight of the wheel will vary in various embodiments from 0.25% to 10%.

The quantity of liquid resin for bonding the solid lubricant will vary from about 5 to 50% of the weight of the solid lubricant suspension.

Where the solid lubricant is put in prior to or along with the resin, or other bonding agent, for making up the abrasive wheel, the wheel bonding materials will constitute between 5 and 40% of the weight of the abrasive wheel.

All percentages relating to compositions stated herein are by weight unless otherwise indicated.

Mesh size is expressed in Tyler standard mesh per linear inch.

5 In view of our invention and disclosure variations and modifications to meet individual whim or particular need will doubtless become evident to others skilled in the art to obtain all or part of the benefits of our invention without copying the method and article of manufacture as shown, and we therefore claim all such insofar as they fall within the reasonable spirit and scope of our claim.

Having thus described our invention what we claim as new and desire to secure by Letters Patent is:

The process of improving the cooling capability of a 15 vitrified bonded abrasive wheel which comprises the steps of preparing a dispersion of graphite powder in isopropyl alcohol wherein the graphite forms about 7% of the dispersion, forming a mixture of the dispersion of graphite powder and isopropyl alcohol with a liquid phenol-formaldehyde resin wherein the phenol-formaldehyde resin comprises about 15% of the mixture, dipping the vitrified bonded abrasive wheel into the mixture and impregnating the mixture within the pores of the wheel, removing the wheel from the mixture and allowing it to 20 drain, and curing the mixture.

#### References Cited by the Examiner

##### UNITED STATES PATENTS

|    |           |         |                      |        |
|----|-----------|---------|----------------------|--------|
| 30 | 1,310,360 | 7/1919  | Martin -----         | 51—295 |
|    | 1,573,061 | 2/1926  | Hartmann -----       | 51—295 |
|    | 2,050,992 | 8/1936  | Aust -----           | 51—295 |
|    | 2,125,782 | 8/1938  | Heald -----          | 51—295 |
|    | 2,367,995 | 1/1945  | Buckey -----         | 51—295 |
| 35 | 2,862,806 | 12/1958 | Nestor -----         | 51—295 |
|    | 2,968,577 | 1/1961  | Helling et al. ----- | 51—295 |
|    | 3,062,633 | 11/1962 | Coes -----           | 51—295 |

ALEXANDER H. BRODMERKEL, Primary Examiner.

40 MORRIS LIEBMAN, Examiner.

D. J. ARNOLD, Assistant Examiner.